

## 1

3,594,326

**METHOD OF MAKING MICROSCOPIC CAPSULES**  
 Rene Karl Himmel, Kilchberg, Switzerland, assignor to  
 The National Cash Register Company, Dayton, Ohio  
 No Drawing. Continuation of application Ser. No.  
 415,809, Dec. 3, 1964. This application Feb. 14,  
 1969, Ser. No. 802,731  
 Int. Cl. B01j 13/02; A61k 9/04; B44d 1/02  
 U.S. Cl. 252—316

2 Claims

**ABSTRACT OF THE DISCLOSURE**

The process of forming minute capsules en masse which comprises (a) establishing an agitated system consisting of a liquid polar vehicle constituting a continuous first phase, a second phase dispersed therein consisting of minute mobile entities of core material, and a third phase dispersed therein consisting of minute, mobile liquid entities of a wall-forming solution of a non-polar polymeric material, the said core material being wettable by said wall-forming solution, the said three phases being mutually incompatible, the third phase constituting such a part of the total three-phase system, by volume that it can exist as a dispersed phase of minute mobile entities capable of and sufficient in amount to deposit around the core entities, and wherein the wall-forming polymeric material has a decreasing solubility with increasing temperature in the vehicle, and wherein the third phase is maintained as such, at least in part, by the presence of a polyelectrolyte polymer (b) hardening the walls so formed by elevating the temperature of the system to a temperature above the gel point of the wall-forming polymer, and (c) separating the hardened capsules from the rest of the system at a temperature above that at which resolution of the capsule walls takes place to any substantial degree.

This application is a continuation of copending application Ser. No. 415,809, filed Dec. 3, 1964, and now abandoned.

This invention relates to a process of manufacturing minute capsules en masse in a liquid manufacturing vehicle and to the capsule product, each capsule comprising a core and a seamless protecting wall surrounding the core. By "minute capsules" are meant capsules, for example, from a few microns to several thousand microns and possibly somewhat larger in average size.

The capsule-forming process of this invention involves the establishment of a system that is characterized as follows (these terms being defined below):

(1) It is in an agitated state;

(2) It comprises the following three phases, characterized first of all by being mutually incompatible (as defined herein) and further characterized, respectively, as follows:

- (a) a continuous liquid phase polar vehicle that constitutes at least a substantial portion by volume of the three phases in total,
- (b) a discontinuous phase of minute, mobile entities of core material, either solid or liquid, dispersed in the vehicle, and
- (c) a discontinuous phase of minute, mobile entities of wall-forming material dispersed in the vehicle and constituted by a liquid solution of a wall-forming polymeric material, said solution being capable of wetting the core material on contact, having a decreasing solubility in the vehicle with a rise in temperature, and said solution preferably having a viscosity greater than the liquid phase vehicle (a), and wherein the wall-forming polymer is non-ionic and there is present in the system a poly-

## 2

electrolyte sufficient in amount to aid in maintaining the wall-forming polymer solution as a separate phase.

This agitated system results without more in a deposit of the solution of the wall-forming polymeric material around the entities of core material. By reason of the ability of polymer solution to wet the core material, and of the viscosity and volume relation of the dispersed phase of wall-forming polymer solution, the dispersed wall-forming polymer solution is capable of deposit around the dispersed entities of core material and also is capable after deposit of maintaining itself as a wall against the shearing forces that exist as an incident of the required agitation of the system. The deposits accumulate to a maximum thickness, which may be varied by varying the amount of the wall material provided and the degree and type of agitation used, which may vary in accordance with the need for protection of the core material and the protective characteristics of the wall-forming material selected for use.

Following deposition of the liquid solution of the wall-forming polymeric material, the temperature of the system is elevated preferably above the gelation temperature of the wall-forming polymer to harden the capsule walls and thereby densify and impart to them greater durability and greater impermeability relative to the core material and the environment, among other properties.

After hardening the capsule walls by elevating the temperature, it is necessary to separate the hardened capsules at a temperature above that at which a substantial amount of the wall-forming polymeric material would be dissolved by the vehicle. If, however, the hardened capsule walls are treated so that they become permanently insolubilized in the vehicle medium, then obviously there is no need for separation of the capsules, and the system may be returned to room temperature without concern that the wall material will be redissolved by the vehicle.

The subject process of making capsules en masse in a liquid polar vehicle by the system defined above utilizes a polyelectrolyte to assist the establishment of the wall-forming polymer solution as a separate phase.

In one form, the process involves forming a solution of the wall-forming polymeric material having the decreased solubility with increase in temperature property noted above in the vehicle and dispersing the core material therein. Upon heating and agitation of the mass, a coacervate solution of the wall-forming polymeric material separates out and deposits about the core material to form embryonic capsules. Continued heating at the same or elevated temperatures effects a hardening of the deposit. Thereafter, separation of the capsules may be carried out at the elevated temperatures, subsequently, the separated capsules are dried.

In another form, the process contemplates adding components to form the system without the necessity of going from a solution of the wall-forming polymeric material to a separated coacervate solution of the polymeric material; i.e. one knowing the relative concentrations of the various components and conditions that will produce a coacervate solution, need only provide such components in the required relative amounts and under conditions that yield a coacervate solution of the polymer. For example, the various components of the system, except the wall-forming polymer, can be brought to a temperature at which it is known that the coacervate solution will form and the wall-forming polymeric material then added to produce a coacervate solution of same and consequent wrapping of the core material with an embryonic shell of wall-forming polymeric material.

In yet another form, a coacervate solution of the wall-forming polymeric material is formed and separated

from its equilibrium liquid. A system for microencapsulation utilizing the separate polymer solution may be had by forming a three-phase system as described above, wherein a liquid vehicle, other than the equilibrium liquid of the coacervate solution, is employed, said liquid vehicle meeting the other criteria of incompatibility set forth herein.

This new process in one respect is an improvement of U.S. Pat. No. 2,800,458 to Green and U.S. Pat. No. 2,800,547 to Green et al., and U.S. Reissue Pat. No. 24,899 to Green et al. in that it provides, in one form, a process directed to a "changing condition" for bringing about coacervation. It is particularly directed to a system wherein the polymeric wall material has a substantial solubility in a solvent, for example, water at room or lower temperature, thus providing an encapsulated material which may be released into a liquid medium at low temperature by dissolution of the capsule wall. A further utility is that core materials having the property of decreasing solubility with increasing temperature may be efficiently encapsulated by the system of this invention. Further, the subject process is an improvement of Baken, U.S. application Ser. No. 413,348, filed Nov. 23, 1964, now abandoned.

It has been discovered that if the polymeric material of the capsule wall possesses the above described solubility characteristic and if the associated liquid of the wall-forming polymer solution and the vehicle are selected to satisfy the further criteria set forth herein, not only is it possible to produce a system in which deposit of the dispersed entities of the solution of the wall-forming polymeric material around particular dispersed core entities can be achieved, but also this can be done with combinations of core materials, wall-forming polymers, and vehicles that could not before be used to successfully encapsulated by en masse microencapsulation techniques.

The further criteria which define the useful classes of materials for the vehicle and the coacervate solution of the wall-forming polymers are these: (1) the liquid wall-forming solution of polymeric materials which form the capsule wall must be capable of wetting the core material in order to deposit around core entities; (2) the solution of polymeric material(s) should have a viscosity, preferably of about 200 to 4000 centipoises, such that it may both deposit and maintain itself deposited around the core entities despite the shearing forces of the agitation needed to maintain the material of the system as a dispersion; (3) the solution of polymeric material(s) preferably constitutes about 5% to 20% by volume of the total three-phase system, so that it can exist as a dispersed phase of mobile entities capable of deposit around the core entities; and (4) the core material, the solution of the polymeric material(s), and the vehicle must be mutually immiscible.

The wetting action of polymeric materials in solution as regards a particular core material may be measured by standard contact-angle measurements, adsorption measurements, and the like, and suitable selections may be made thereby, all in accordance with existing knowledge of this subject per se. The solvent for the polymeric materials(s) may in certain instances be selected to enhance the wetting action of a particular polymeric material solution with respect to a chosen core material.

The stated criterion that the core material, the polymeric material solution, and the vehicle be mutually incompatible is used in the sense that their separate existence in the system must not be impaired by a reactivity or miscibility between them.

Prefabricated incomplete systems for use in carrying out the novel process may be established and stored for future use. Even unskilled operators may complete such systems by the addition of the missing components, with the required agitation and heat, together with the agents for hardening of the walls, to make capsules at a later

time. The missing component(s) may involve any of those three necessary to form an operative system, and the absence may be total or partial.

Whether the liquid solution of wall-forming polymeric material is formed by effecting a phase separation or by adding components in proper amount to create said solution without need for phase separation, the agency that causes or maintains the separation of the wall-forming polymer solution may be one or more "changing conditions" including as an essential condition the presence of a sufficient amount of polyelectrolyte. In the usual case the insolubility of the wall-forming polymer with increasing temperature will be employed as a "changing condition" in conjunction with the polyelectrolyte. Illustrative of "changing conditions" which may be used alone or in combination with the addition of polyelectrolyte to the mass is the presence of a non-solvent for the wall-forming polymer which is compatible with the vehicle, or other known techniques that provide a "changing condition" to effect or maintain a separation of the wall-forming polymer solution, such as, for example, change in micro-ion concentration (salt, pH), all of which are techniques employed to bring about separation of a coacervate solution.

The preferred system is one in which the liquid associated with the wall-forming non-polar polymer solution also is used as a major component material of the manufacturing vehicle and wherein there is present as a component as polyelectrolyte polymer which may or may not possess the property of decreased solubility with increased temperature and which is complementary to the wall-forming polymer in the sense that it assists in creating an incompatibility between the vehicle and the solution of the wall-forming polymeric material(s) and induces or maintains the solution as a separate phase in the system. In other words, it completes a liquid system in which the wall-forming solution of polymeric material can exist as a separate phase, which may be dispersed in the vehicle by agitation, because of repulsive forces between the polymeric material of the wall-forming solution and the complementary material. Without the complementary polyelectrolyte polymeric material, if the vehicle included or consisted of the same liquid that is used as the solvent of the wall-forming polymeric solution, the vehicle would be more compatible with and would dilute the polymer solution. Thus, the stated incompatibility between the vehicle and the solution of wall-forming polymeric material connotes the presence of a complementary material as a constituent of the vehicle when the vehicle includes a liquid compatible with or identical to the solvent used in the wall-forming coacervate solution.

The nature of the core material is the primary guide to the selection of the particular non-polar polymeric wall-forming material and of its polar solvent, and also to the selection of the liquid vehicle if that is not to consist of or include as a component the same material that is used as the wall-forming polymer solvent. This is because the process conditions usually are chosen with the object of encapsulating some given core material. Hence the wall-forming polymeric solution must be incompatible with the core material, but capable of wetting and depositing around entities of it. The wall-forming polymeric material may be hydrophobic; again the nature of the core material and the requirement that core material and wall-forming material be incompatible dictating the choice of non-polar polymeric material. In the preferred system from the class of polymers and solvents made eligible by these criteria, the further choice is from among those polymer-solvent pairs which can form a wall-forming polymer solution. When, as preferred, the vehicle is made up chiefly or wholly of the same material as the polymer solvent, the only further choice is, in the preferred embodiment, with respect to the complementary material (polyelectrolyte polymer), which again, must meet the incompatibility requirement. The complementary material

must be incompatible with the core material and must act to make the wall-forming non-polar polymeric material solution more incompatible with the vehicle.

Given these criteria of selection, not known before in total as the determinants of an operative encapsulation system, the classes of materials that are useful in constituting the polar vehicle and the solution of the non-polar wall-forming polymer of the present system are ascertainable from existing knowledge and means of selection of polymeric materials and solvents in respect of four properties; viz:

- (1) solubility of the polymeric material in various solvents;
- (2) ability of the non-polar polymeric material solution to wet the given nucleus material, liquid or solid;
- (3) the temperature-solubility characteristics of the non-polar polymeric material; and
- (4) ability of a solution of the non-polar polymer to exist in a separate solution phase in the vehicle liquid.

Materials thus selected are useful in the encapsulation of any incompatible and wettable core material, liquid or solid.

#### POLYMERIC MATERIAL

Examples of hydrophilic, non-polar wall-forming polymeric material which possess the property of decreased solubility with increasing temperature include methyl cellulose, polyvinylmethyl ether, and ethylhydroxyethyl cellulose. An example of suitable hydrophobic wall-forming polymeric material is nitrocellulose.

Examples of hydrophilic polyelectrolyte polymeric material which are complementary to the wall-forming polymer and assist in establishing the wall-forming polymer solute and carboxymethylcellulose, sodium carboxymethylcellulose, and gum arabic.

#### SOLVENTS

Water may be used as the solvent of the wall-forming solution in the instances where the wall-forming polymer is hydrophilic, organic polar solvents where the polymeric material is hydrophobic. Obviously, the choice of solvent is dependent upon the solubility of the wall-forming polymer therein. Preferably, where the encapsulation involves a phase separation the solvent should be one wherein the polymer is reasonably soluble at room temperature, so that upon elevation there will be sufficient polymer available for phase separation and deposit about the core material.

In general, the decrease in solubility with increase in temperature of the wall-forming polymeric material can be affected by appropriate selection of the polymer and solvent. The solvent ability varies with both the size and shape of the solvent molecules. As a rule small solvent molecules are better solvents at elevated temperatures than lower temperatures, whereas with large solvent molecules the reverse is true.

#### CORE MATERIALS

Core materials may be any substance that survives separately in the system but those for which the process of the subject invention is particularly suited are, as stated above, those materials which are insoluble in the vehicle phase, for example, such as, chloroform, Aroclor (chlorinated biphenyl), kerosene, mynacet(acetylated monoglyceride), lemon oil, menthol, aspirin, resins, pigments and dyes.

In its broader aspect, the invention is not in the discovery of particular polymeric materials or solvents or vehicles but rests on and applies to the discovery that liquid and solid core materials can be encapsulated as nuclei in an agitated fluid system by utilizing a polyelectrolyte complementary to and lessening the solubility of wall-forming polymeric material in a polar liquid.

The proper volume relation of the wall-forming phase (of proper viscosity) can be predetermined to a close 75

enough approximation by calculation from readily-ascertained data on the relation of viscosity to concentration for a solution of the intended wall-forming polymeric material in the chosen solvent.

5 The order of addition can be reversed, or the two polymeric materials and the solvent can be brought together at one time, once the proper quantitative relations are established for the particular materials being used, since the resulting volume and viscosity (concentration) of the 10 two separate phases are independent of the order of assembly.

The core material, always a minor component of the total volume of the system, can be added either before or during or after the formation of the solution into two 15 solution phases. Similarly, the agitation of the system can be begun before, during, or after either of these steps. It is preferred, however, to agitate before, during and after the phase separation, and to introduce the core material after the phase separation has taken place.

20 The intensity of the agitation is made such as to reduce the core material to the desired entity size, if such is necessary, and, in any event, to assure thorough dispersion of it in the vehicle. The core entity size is pre-selected to give the desired capsule size after allowance 25 for encapsulating wall thickness. With solid core materials, the entity size can be predetermined and obtained by any suitable grinding or milling.

In the following example, the novel process will be disclosed in detail as applied to the encapsulation of various 30 materials. The example illustrates the sequence of steps in an application of the invention employing a non-ionic polymer and a polyelectrolyte.

(1) Into 100 grams of an aqueous 2% methylcellulose solution is thoroughly stirred 10 grams of the water insoluble material or nuclei to be encapsulated either in the 35 form of powder or as a liquid in which case the mixture is stirred until the material is thoroughly emulsified to the requisite drop size.

(2) In this solution, and whilst stirring, is thoroughly 40 mixed 100 grams of a 2% aqueous solution of carboxymethylcellulose.

(3) The mixed solution is now heated to about 60° C.

(4) At any time during the heating 300 ccs. of a 20% solution of sodium chloride or sulphate or ammonium 45 chloride or sulphate is added.

(5) The heating is continued for about 1 hour during which the polymers separate out to form homogeneous and continuous coatings separately round the nuclei thus to preform the capsules.

(6) Whilst still warm the separated phase is segregated 50 by decanting the supernatant or by filtration.

(7) The segregated phase is now dried in an oven or by hot air blast to drive off the remanent water in the capsule walls which results in a dry freely flowing powder like residue composed of individual capsules with the walls consisting of the two polymers in a complex admixture. The walls may be hardened or plasticized.

What is claimed is:

1. The process of forming minute capsules en masse which comprises the steps consisting essentially of

60 (a) establishing an agitated system consisting of first, second and third liquid phases, said system consisting of a liquid polar vehicle constituting a continuous first phase, said first phase having dispersed therein a polyelectrolyte polymer, a second phase dispersed therein consisting of minute mobile entities of core material, and a third phase dispersed therein consisting of minute, mobile liquid entities of a wall-forming solution of methylcellulose; further the said core material being wettable by said wall-forming solution, the said three phases being mutually incompatible, and the third phase constituting such a part of the total three-phase system by volume, that it can exist as a dispersed phase of minute mobile entities capable of and sufficient in amount to de-

- posit around the core entities; and further wherein the third phase is formed by elevating the temperature of the system to cause the emergence of a coacervate solution of methylcellulose and said third phase is maintained as such, at least in part, by the presence of a polyelectrolyte polymer which is complementary to methylcellulose,
- (b) hardening the walls so formed by elevating the temperature of the system to a temperature above the gel point of methylcellulose, and
- (c) separating the hardened capsules from the rest of the system at a temperature above that at which resolution of the capsule walls takes place to any substantial degree.
2. The process of claim 1 wherein during the formation of the third phase the system is heated to a temperature

5

10

15

above room temperature but below the gel point of the methyl cellulose to thereby assist in the formation of the third phase by causing the coacervate solution of the methyl cellulose solution to emerge.

#### References Cited

##### UNITED STATES PATENTS

3,242,051 3/1966 Hiestand et al. \_\_\_\_ 252—316X  
3,244,640 4/1966 Studt et al. \_\_\_\_\_ 252—316

RICHARD D. LOVERING, Primary Examiner

U.S. CL. X.R.

99—118, 140, 166; 117—100; 264—4; 424—33, 34, 35.  
343